

Patented Feb. 26, 1929.

1,703,693

## UNITED STATES PATENT OFFICE.

GINO M. ROSSATI, OF PADUA, ITALY, AND GIUSEPPE DE BLASIO, OF NEW YORK, N. Y.

## ARTIFICIAL WOOL.

No Drawing.

Application filed January 18, 1928. Serial No. 247,744.

This invention relates to a new and useful method of preparing vegetable fibres so that they resemble natural wool in appearance, texture, strength, and in other respects.

5 In accordance with our process the medium to be converted is a vegetable fibre, preferably one belonging to the family of "Tiliaceæ." The plant belonging to this family which we find most suited to our purpose is jute. The jute fibres to be converted are first immersed in a bath of lime water of the concentration of 1%. The period of immersion should be fairly long and we have found that about two hours are required to 10 obtain best results. In immersing the jute in this bath care should be taken that it be suspended in the bath or otherwise kept out of contact with the sediment which is usually found at the bottom of the vessel containing 15 the lime solution. The jute is then removed from the bath and, without previous drying, is subjected to the action of sulphur dioxide for about one hour, after which the fibre is allowed to rest for about twelve hours. Subsequently the fibre is washed and dehydrated, 20 preferably in a centrifuge.

The above described treatment of the fibre is for the purpose of detaching and dissolving the combs that normally keep the fibres 25 united.

After removal from the centrifuge the fibre is treated directly with a caustic solution of suitable concentration, preferably a solution of caustic soda at 10 Bé., whereupon it is kept 30 until almost perfectly dry. The treatment with the caustic soda and the subsequent drying of the fibre is for the purpose of strengthening the fibres and causing them to crinkle so that the ultimate product may readily be 35 mixed and woven into cloth with natural wool.

40 As the next step in the process, the fibre is thoroughly washed in water and then placed in a bleaching solution such as a bath of sodium perborate, hydrogen peroxide or 45 sodium hypochlorite. The fibres are then washed in water to which 1/4% of sodium bisulphite has been added for the purpose of "fixing" the washing process. Then the fibres 50 are washed in acidulated water, preferably a solution of 1/2% hydrochloric acid or sulphuric acid being used for that purpose. This will clean off all caustic soda that may 55 remain on the fibres. The fibres are then immersed in a bath of sulphonated fatty acid which will lubricate the fibres and give them

the necessary suppleness and texture. Finally, the fibres are dried without any washing and will have the aspect of natural wool and can be used in substantially the same manner.

60 It will be obvious to those skilled in the art that the process may be practiced with various modifications within the scope of the invention which is defined in the claims.

## What we claim is:

1. The method of preparing vegetable fibres so that they resemble in quality natural wool, characterized by the step of immersing the fibres in a clear solution of lime water.

65 2. The method of preparing vegetable fibres of the family of Tiliaceæ so that they resemble in quality natural wool, characterized by the step of immersing the fibres in a bath of lime solution free from undissolved lime.

70 3. The method of preparing vegetable fibres so that they resemble in quality natural wool, which comprises the following steps: immersing the fibres in a bath of lime water, subjecting them to the action of sulphur dioxide, allowing the fibres to rest, treating the fibres with a caustic solution, and immersing the fibres in a bath of sulphonated fatty acid.

75 4. The method of preparing vegetable fibres so that they resemble in quality natural wool, which comprises: destroying the combs which unite the fibres, washing said fibres, treating the fibres with a caustic solution and then drying them to crinkle the fibres, fixing the washing process, removing all caustic from the fibres, lubricating the fibres, and finally drying the fibres.

80 5. The method of preparing vegetable fibres so that they resemble in quality natural wool, which comprises: immersing the fibres in a bath of lime water out of contact with the sediment in the bath, subjecting them to the action of sulphur dioxide, allowing the fibres to rest, washing and dehydrating said 85 fibres, treating the fibres with a caustic solution, placing the fibres in a drying chamber until almost perfectly dry, fixing the washing process, removing all caustic from the fibres, lubricating the fibres, and finally drying the 90 fibres.

95 6. The method of preparing vegetable fibres so that they resemble in quality natural wool, which consists in immersing the fibres in a bath of lime water of a concentration of 1% out of contact with the sediment in the 100 bath for a period of two hours, subjecting 105 the fibres to the action of sulphur dioxide, allowing the fibres to rest, washing and dehydrating said fibres, treating the fibres with a caustic solution, placing the fibres in a drying chamber until almost perfectly dry, fixing the washing process, removing all caustic from the fibres, lubricating the fibres, and finally drying the 110 fibres.

them to the action of sulphur dioxide for a period of about one hour, allowing the fibres to rest for a long period of time, washing and dehydrating said fibres, treating the fibres 5 with a caustic solution at 10 Bé., again dehydrating the fibres, placing the fibres in a drying chamber until almost perfectly dry, placing them in a bleaching solution, again washing the fibres in water containing a  $\frac{1}{4}\%$  of 10 sodium bisulphite solution, washing the fibres in acidulated water, immersing the fibres in a bath of sulphonated fatty acid, and finally drying the fibres.

7. The method of preparing jute fibres so 15 that they resemble in quality natural wool, which consists in immersing the fibres in a bath of lime water of a concentration of 1% out of contact with the sediment in the bath for a period of two hours, removing the fibres 20 from the bath and without previous drying subjecting them to the action of sulphur dioxide for a period of one hour, allowing the fibres to rest for a period of about 12 hours, washing and centrifuging said fibres, treating

the fibres with a solution of caustic soda at 25 10 Bé., again centrifuging the fibres, placing the fibres in a drying chamber until almost perfectly dry, thoroughly washing the fibres, placing them in a bleaching solution, again washing the fibres in water containing 30  $\frac{1}{4}\%$  of sodium bisulphite solution, again washing the fibres in water acidulated with  $\frac{1}{2}\%$  hydrochloric acid, immersing the fibres in a bath of sulphonated fatty acid, and finally drying the fibres. 35

8. The method of preparing vegetable fibres so that they resemble in quality natural wool, which comprises treating the fibres with a clear solution of lime water, then with a solution of caustic alkali and then with a fixing solution, and washing the fibres after each 40 of the above treatments.

In testimony whereof, we have signed our names to this specification, this 17th day of January, 1928.

GINO M. ROSSATI.  
GIUSEPPE DE BLASIO.